

Nov. 15, 1938.

J. A. BOYER

2,137,201

ABRASIVE ARTICLE AND ITS MANUFACTURE

Filed June 28, 1937



INVENTOR.  
JOHN A. BOYER

BY

*R. A. Beemer*  
ATTORNEY.

## UNITED STATES PATENT OFFICE

2,137,201

## ABRASIVE ARTICLE AND ITS MANUFACTURE

John A. Boyer, Niagara Falls, N. Y., assignor to  
The Carborundum Company, Niagara Falls,  
N. Y., a corporation of Delaware

Application June 28, 1937, Serial No. 150,766

3 Claims. (Cl. 51—280)

This invention relates to metal bonded abrasive articles and their manufacture, and particularly to the metal bonding of such abrasives as silicon carbide, boron carbide, fused alumina 5 and diamonds.

One of the objects of the invention is to produce a metal bonded abrasive article having improved grinding or lapping characteristics. Another object of the invention is to produce 10 a metal bonded abrasive article in which the bond or matrix is characterized by high degree of coherence and strength, and in which the bonding material can be matured at a relatively low temperature. A further object is to produce 15 a metal bond or matrix for abrasives in which the coalescence of the metal particles is facilitated by comparative freedom of the metal from surface films of oxide. A further object is to provide a metal bond or matrix which will satisfactorily retain the abrasive during lapping or 20 grinding, but which can be readily dressed so as to present a free cutting surface. These and other objects will be apparent from the present specification.

In the bonding of abrasives with metal, it is 25 difficult to provide a metal or alloy which has the characteristics required for a satisfactory abrasive bond. The non-metallic materials used for bonding abrasives are brittle, and efforts in connection with metal bonding have been directed principally towards duplicating this property by the use of hard or brittle materials. When the bond or matrix is extremely hard, it is 30 difficult to dress the wheel after the abrasive becomes worn, so that a fresh cutting surface cannot readily be presented. When the bond or matrix is brittle, it chips out upon grinding with consequent loss of abrasive. A brittle matrix has the further disadvantage that when the 35 abrasive content is increased so as to become a major portion of the wheel, the bond or matrix is weakened by the discontinuous structure caused by the presence of the abrasive particles. In metal bonded wheels having a high abrasive 40 concentration or in wheels in which extremely fine grits are employed, it is necessary to provide a strong metallic structure throughout the wheel if any advantage is to be derived from the use of metal as a bonding agent.

In the production of metal bonded abrasives, 45 I have found that silver and silver alloys possess very desirable bonding characteristics. Silver has no affinity for oxygen at high temperatures, and as the particles of silver are entirely free 50 from oxide films, the powder sinters readily into a coherent mass and at the same time retains the abrasive so as to produce a wheel having a high cutting efficiency. Other metals diffuse rapidly into silver when the metal is heated to 55 temperatures substantially below its melting

point, so that sintered alloys can be readily formed from a mixture of the component metal powders. Silver also has a very high thermal conductivity, and any localized heat generated during cutting or grinding is rapidly conducted 5 to the cooler portions of the wheel. The high thermal conductivity of the wheel is of particular importance in the cutting or lapping of such materials as glass and quartz, which chip very readily. I have found that with silver bonded 10 wheels, it is possible to retain a very fine edge and cut extremely thin sections of these materials without chipping. With silver bonded 15 wheels I have been able to cut very thin sections of quartz for radio frequency apparatus where even the slightest degree of localized heating will crack the section being cut.

For the cutting of glass and other materials which have a dressing action on the wheel, it is 20 possible to use a very ductile matrix such as pure silver, providing sufficient abrasive is present in the wheel to prevent rapid wearing away of the metal matrix.

In abrasive articles in which diamonds are 25 bonded with silver or silver alloys, the wear resistance of the matrix can be substantially increased by the addition of particles of other abrasives such as boron carbide, silicon carbide or fused alumina. This additional abrasive material, even though it may do practically no cutting in comparison with the cutting done by the 30 diamonds, stiffens the metal matrix and makes it more resistant to wear and abrasion. The diamond content can thus be reduced to a relatively low percentage and the wheel will still 35 have a satisfactory cutting rate and a long life.

Although pure silver forms a satisfactory bond 40 for many purposes, it is usually desirable to harden the silver by the addition of alloying agents. Silver has the property of retaining a 45 number of metals in solid solution, i. e., in homogeneous admixture therewith in the solid state, up to fairly high percentages, and the resulting alloys are hard, strong and ductile. Another group of alloys in which only a part of the alloying ingredients are retained in solid solution, namely, alloys of silver, copper and zinc or cadmium, which will be further described, have a strength approaching that of mild steel, the ductility of brass or bronze, the resistance to 50 oxidation of a heat-resistant alloy and melting points as low as 700 to 750° C. I know of no other metallic materials possessing this combination of properties. When alloys of this type are used for the bonding of the abrasive particles, they satisfactorily retain the abrasive and 55 provide a metal matrix having a very high degree of coherence and strength. The low sintering or melting temperatures are of particular advantage in the commercial production of 60

bonded abrasives, especially in the case of combustible or readily oxidizable abrasive materials such as the diamond.

The exact nature of the invention will be more clearly understood from a consideration of the accompanying drawing.

In the drawing:

Figure 1 shows an equilibrium diagram of the silver-copper alloys from 0 to 100% silver;

Figure 2 shows an equilibrium diagram of the silver-cadmium alloys from 0 to 61% cadmium, which is typical of the equilibrium relations of alloys in which silver retains a high percentage of another metal in solid solution;

Figure 3 shows a plan view of an abrasive wheel in which the periphery contains diamonds and the inner portion of the wheel is composed of metal and an abrasive other than diamonds;

Figure 4 shows a section of a wheel which is adapted for the facing of tungsten carbide tool points by side grinding; and

Figure 5 shows a plan view of the wheel illustrated in Figure 4.

The effect of the copper upon the melting temperatures and the sintering temperatures of the silver-copper alloys may be understood from the equilibrium diagram of this alloy series, which is shown in Figure 1.

Although copper has a higher melting point than silver, it reduces the melting point of the silver when added to it as an alloying ingredient. The copper also has a moderate hardening effect, and produces a bond which is somewhat harder than pure silver and at the same time is free from brittleness. In the diagram, the temperature of complete melting of the silver-copper alloys is represented by the curve 2 and the temperature of incipient melting is shown by the line 3. For practically all alloys of the series this incipient melting point is 778° C., as compared with 932° C. for the melting point of pure silver. Most of the alloys melt over a range of temperatures but the alloy containing 72% silver has a constant melting point of 778° C.

In making a metal bonded abrasive from a silver-copper alloy containing a high percentage of silver, it is desirable to use the eutectic composition containing 28% copper. The metals can be previously alloyed and then comminuted to powder, and upon pressing and heating, the bond will soften and coalesce at the temperature below 778° C. If it is desired to completely melt the bond, melting will take place when a temperature of 778° C. is reached or exceeded, as is indicated by the point 4 on the diagram shown in Figure 1.

An alloy bond or matrix of the eutectic composition can also be prepared by mixing the component metals in powdered form with the abrasive and subsequently applying heat and pressure. The articles can be pressed during the heating process or they can be cold molded and subsequently heated to a temperature slightly below 778° C. If a molten bond is desired, the temperature of 778° C. can be exceeded.

Silver can retain zinc and cadmium in solid solution up to fairly high percentages, and these solid solutions provide bonds which are harder than pure silver but at the same time are ductile. The partial equilibrium diagram of the silver-cadmium alloy is shown in Figure 2. In this figure the temperatures of incipient melting and of complete melting are represented by the curves 6 and 7 respectively. All compositions up to about 37% cadmium are ductile solid solutions

of the type ordinarily designated in metallurgical practice as "alpha" solid solutions. In solid solutions of this type, a pure metal forms the basis for the lattice structure as determined by X-ray diffraction, and the addition of the second metal merely produces a change in the lattice dimensions without producing an undissolved constituent. After the composition of 37% cadmium is reached, a second metallic constituent appears which is harder than the solid solution and which can act as an additional hardening agent. This material is, however, brittle and the brittleness of the alloy increases as the cadmium content is increased.

Silver can also retain zinc in solid solution up to about 25%, and the "alpha" solid solution is characterized by properties similar to that of the "alpha" solid solution of cadmium. The ternary alloys of silver, zinc and cadmium have the same general properties. As previously pointed out, it is possible to exceed the solid solubility limit in these alloys and obtain a further hardening effect by the production of a second constituent without producing extreme brittleness. The addition of copper in amounts of, for example, from 5 to 10% to these alloys also produces further hardening. With higher additions of copper, the alloys become relatively low melting, and come within the general classification of silver solder.

The following are examples of silver solders which form suitable abrasive bonds or matrices. These alloys are particularly adapted for the bonding of diamonds because of their extremely low melting points combined with high strength. Owing to the relatively high silver content of the alloys, they can be sintered into a coherent mass from powder at temperatures which have no injurious effect upon the diamond.

| Silver | Copper | Zinc | Cadmium | Phosphorus | 40 |
|--------|--------|------|---------|------------|----|
| 80     | 15     | 5    | --      | --         |    |
| 75     | 20     | 5    | --      | --         |    |
| 70     | 30     | --   | --      | --         |    |
| 65     | 29     | 15   | --      | --         |    |
| 65     | 20     | 9    | 5       | --         | 45 |
| 65     | 20     | --   | 15      | --         |    |
| 60     | 25     | 15   | --      | --         |    |
| 50     | 15     | 15   | 15      | 5          |    |
| 50     | 15     | 15   | 20      | --         |    |
| 40     | 36     | 24   | --      | --         | 50 |
| 25     | 70     | --   | --      | 5          |    |

Silicon can also be added to pure silver or to silver alloys to produce a hardening effect upon the abrasive bond. When silicon is added to pure silver it does not form an intermetallic compound, and the resulting alloy consists of silicon particles embedded in a continuous silver matrix. The juncture between the surface of the silicon particles and the silver matrix is, however, a true alloy joint. Since the silver matrix is practically continuous a substantial hardening effect can be obtained without causing a high degree of brittleness. Compositions of, for example, from 5 to 40% silicon can be used. When silicon is added to silver alloys containing copper or other metals which form silicides, the resulting compound formed with the silicon, although hard, has a tendency to be brittle, and the properties of the bond can be controlled over fairly wide limits by the introduction of these brittle compounds of silicon in various proportions.

The alloys of silver and copper with phosphorus are low melting, and have properties

similar to those of the silver solders containing zinc or cadmium.

- In bonding silicon carbide or fused alumina with silver alloys, or in the bonding of diamond or boron carbide for purposes where an extremely high cutting rate is necessary, it may be desirable to employ an alloy having brittle characteristics. Such alloys can be produced from silver by appreciably exceeding the solid solubility limits (as for example in the case of zinc and cadmium), by the production of brittle intermetallic compounds such as the silicides by the addition of silicon in fairly high percentages, or by the addition of arsenic and antimony which can be added in minor proportions either to silver or to the above described alloys. Silver sulphide is also soluble in silver, and an "alloy" of silver and silver sulphide will produce an embrittling effect when it is desired to obtain a brittle bond.
- The addition of tin to silver in minor percentages (as for example from 5 to 20%) also produces a satisfactory abrasive bond or matrix. If the bond is made from comminuted component metals, the tin upon heating melts at 232° C. and diffuses into the silver so as to form an alloy. This melting and subsequent diffusion, resulting in re-solidification at higher temperatures, facilitates the coalescence of the powdered metal into a homogeneous matrix or bond.
- Methods of making an abrasive wheel of the type shown in Figures 3, 4 and 5 can be illustrated by specific examples, although it will be realized that these examples are merely illustrative and are not intended to be limiting in regard to alloy compositions, grit sizes or methods of molding and sintering.

#### Example I

A peripheral grinding wheel of the type shown in Figure 3 can be made as follows:

A cylindrical mold is separated into an inner and an outer compartment with a paper separator, the width of the outer compartment being that desired for the rim 9 containing the cutting abrasive. Into this outer portion of the mold is placed a mixture of 7 per cent diamonds, 10 per cent silicon carbide, 25 per cent copper powder, and 58 per cent silver powder. The diamonds can be from 100 to 200 grit; the silicon carbide from 180 to 600 grit, and the metal powder finer than 200 mesh. The inner space within the mold is filled with a mixture of 20 per cent silicon carbide, 24 per cent copper powder and 56 per cent silver powder, using approximately the same particle sizes as in the outer rim. The mixes in the respective compartments are levelled off, the paper separator removed, the mix again levelled, and subjected to pressure of, for example, from 10,000 to 50,000 lbs. per square inch. The pressed wheel is then removed from the mold, and is sintered in a non-oxidizing atmosphere at a temperature of 700 to 750° C. The wheel may be placed between two ceramic bats and sintered under a slight pressure to prevent warping.

#### Example II

A wheel for the side grinding of tungsten carbide tools, such as is illustrated in Figures 4 and 5, can be made as follows:

A composite abrasive ring is molded by first placing in a ring-shaped mold a mixture of 10 per cent diamonds of 100 to 200 grit, 10 per cent silicon carbide of from 180 to 600 grit, 52 per cent silver powder, 16 per cent copper powder, and 12 per cent zinc powder. This mixture is levelled

off, and a backing mixture composed of 75 per cent copper powder and 25 per cent of silicon carbide of a grit size corresponding approximately to the grits used in the abrasive layer. The backing layer is levelled off, and the composite ring subjected to a pressure of from 10,000 to 50,000 lbs. per square inch. The wheel is then sintered to a temperature of approximately 700° C.

#### Example III

A previously alloyed silver solder containing 60 per cent silver, 25 per cent copper and 15 per cent zinc is cocomminuted to powder. The metal powder is mixed with abrasive grain in the desired proportions, as for example, with from 5 to 20 per cent diamonds, with diamonds and an abrasive of a lesser degree of hardness as described in the two previous examples, with boron carbide mixed with silicon carbide or fused alumina, or with boron carbide, silicon carbide or fused alumina alone. In using silicon carbide or fused alumina, the abrasive content can be increased to fairly high percentages if desired. The article can then be molded and sintered by any suitable method, as for example, by the methods described in detail in the previous examples. As an alternative to the molding of the material while cold under a high pressure, the abrasive mix and the mix for the metal backing can be introduced into a carbon mold and the composite ring sintered under pressure. It is possible by this method to sinter an abrasive mix directly onto a solid metal backing.

In the wheel shown in Figure 3, only the outer rim or periphery 9 is used for grinding. It is desirable however, to add a quantity of abrasive or other inert filler material in the inner portion 10 of the wheel so as to make the shrinkage of the inner part of the wheel comparable with the outer ring which is intended to do the cutting. This equalization of shrinkage tends to minimize warping during the sintering process.

In the wheel shown in Figures 4 and 5, the cutting layer 12 consists of an abrasive and a matrix of sintered metal. When the wheel is to be used for the cutting of such materials as tungsten carbide tools, glass or silicon carbide, it is desirable that the abrasive layer contain a certain percentage of diamonds as, for example, from 5 to 10%. As the abrasive layer is comparatively thin, it is advisable in molding the ring 12 to mold thereto a backing 13 of metal powder containing no diamonds. It is also desirable to add a cheap abrasive or a filling material to the backing in order to minimize warping during curing. After the ring is sintered it can be mounted on any suitable backing 14, such as for example, a backing of a reversible thermoplastic resin. If it is desired, the backing 14 can be made of metal and the ring soldered or otherwise attached thereto.

In making an article of high abrasive content from materials such as boron carbide, silicon carbide, fused alumina, the article can be preformed from a mixture of abrasive grains and a suitable binder, and then impregnated with silver or a silver alloy. This impregnation can be carried out by surrounding the article with solid metal, and heating the two materials under vacuum or reduced pressure until the silver or the alloy melts and permeates the pores of the abrasive article. A material of this nature is practically non-porous and the silver forms a tough supporting matrix for the abrasive. If the abrasive particles are very finely divided, the material formed is suffi-

ciently homogeneous so that it can be used for bearings, tool tips and other similar purposes. Diamonds can be admixed with the principal abrasive if desired, or the diamonds themselves can be formed into a shaped article and impregnated.

For the impregnation of abrasive bodies which are self-bonded or which will withstand a very high temperature, the article can be surrounded with solid or liquid metal, and the temperature of the article rapidly raised until the metal flows into the pores of the article at atmospheric pressure. With "recrystallized" or self-bonded silicon carbide, this temperature is about 1900° C. Silver has a unique advantage for this purpose, in that it forms neither a silicide nor a carbide, whereas practically all other metals combine with either one or both of these elements, and when used to impregnate silicon carbide form either brittle silicides or unstable carbides.

The abrasive wheels shown in the drawing are merely illustrative examples, and other types of abrasive articles such as lens grinding laps, cup wheels for the surfacing of glass and refractory shapes, cut-off wheels for glass, tungsten carbide and other hard substances, drills, insert teeth for stone saws, and wheels for petrographic thin sections, can be produced by the process herein described.

By the term "silver base alloy" as used in this specification and the appended claims is meant an alloy of silver and one or more other alloy ingredients, in which alloy silver is the predominant metal.

By the term "eutectic alloy" as used in this specification and the appended claims is meant the alloy solidifying at constant temperature having the lowest melting point of the system.

By the term "solid solution" as used in this specification and the appended claims is meant an alloy constituent in which the crystals of one metal in separating from the liquid contain appreciable amounts of some other metal or compound. The crystals of such a constituent are homogeneous, are not themselves compounds, and cannot be resolved into different constituents under the microscope.

The invention can be defined as being within 10 the scope of the following claims:

1. An abrasive article consisting of abrasive material comprising diamonds embedded and dispersed in a sintered metal matrix consisting principally of a ductile silver-base alloy which alloy 15 contains as a hardening agent at least one metal other than silver retained in solid solution, in such an amount as to harden the matrix but not to destroy its ductility.

2. An abrasive article consisting of abrasive 20 material comprising diamonds embedded and dispersed in a sintered metal matrix consisting principally of a ductile silver-base alloy which alloy 25 contains copper as a hardening agent retained in solid solution, in such an amount as to harden the matrix but not to destroy its ductility.

3. An abrasive article consisting of abrasive material comprising diamonds embedded and dispersed in a sintered metal matrix composed of a ductile alloy consisting principally of silver and 30 containing, at least in part in solid solution, as hardening alloying materials, copper and a metal of the group consisting of zinc and cadmium, in such amounts as to harden the matrix but not to destroy its ductility.

JOHN A. BOYER.

35